# EUROPEAN PATENT SPECIFICATION

(11) **EP 2 623 626 B1**
(45) Date of publication and mention of the grant of the patent: **20.11.2019**
(21) Application number: 11827949.6
(22) Date of filing: 14.04.2011
(51) Int. Cl.: C22C 38/06, C21D 8/12, C21D 8/02, B22D 11/18, B22D 11/22, C21D 6/00, C22C 38/00, C22C 38/02, C22C 38/04, H01F 1/16

(54) **NON-ORIENTED ELECTRIC STEEL PLATE WITHOUT CORRUGATED FAULT AND PRODUCTION METHOD THEREOF**
NICHTORIENTIERTE ELEKTRISCHE STAHLPLATTE OHNE WELLUNGSFEHLER UND HERSTELLUNGSVERFAHREN DAFÜR
TÔLE D'ACIER ÉLECTRIQUE NON ORIENTÉE EXEMPTE DE DÉFAUT D'ONDULATION ET SON PROCÉDÉ DE PRODUCTION

(30) Priority: 30.09.2010 CN 201010298965
(43) Date of publication of application: 07.08.2013
(73) Proprietor: Baoshan Iron & Steel Co., Ltd., Shanghai 201900 (CN)
(72) Inventor: ZHANG, Feng, Shanghai 201900 (CN); CHEN, Xiao, Shanghai 201900 (CN); CAO, Wei, Shanghai 201900 (CN); SUN, Yezhong, Shanghai 201900 (CN); MA, Changsong, Shanghai 201900 (CN); ZHU, Jianru, Shanghai 201900 (CN); CHEN, Zhuolei, Shanghai 201900 (CN); LIU, Xiandong, Shanghai 201900 (CN)
(74) Representative: Copsey, Timothy Graham
(86) International application number: PCT/CN2011/072766
(87) International publication number: WO 2012/041053

(56) References cited:
- EP-B1- 1 346 069
- EP-B1- 1 501 951
- WO-A1-03/097884
- WO-A1-2006/068399
- CN-A- 1 548 569
- CN-A- 1 611 616
- CN-A- 1 611 616
- CN-A- 1 796 015
- CN-A- 1 887 512
- CN-A- 1 887 512
- CN-A- 100 999 050
- JP-A- S 532 332
- US-A- 4 066 479
- US-A1- 2008 121 314

## Description

### Technical Field

The present invention relates to a non-oriented electrical steel sheet and a manufacturing method thereof, especially to a middle steel grade non-oriented electrical steel sheet without corrugated defect, which has an excellent magnetism, and a manufacturing method thereof.

### Description of the Prior Art

For a non-oriented electrical steel sheet having a high extent of silicon, in the surface of a finished strip, accidented waves, similar to corrugations, appear in a direction of rolling, which is generally called "corrugated defect". This defect will reduce a stacking coefficient of the finished strip notably, making the magnetism of the finished strip worse and the electrical resistance between insulating film layers decreased, thus reducing the service performance and life of terminal production. Therefore, almost all of users have a definite demand that a finished strip having corrugated defects is not allowed.

The mechanism of the generation of the corrugated defects may be explained as follows: the equiaxed crystal ratio in the slab is low, whereas the columnar crystal is gross and growing. The growing direction of the columnar crystal <001>, which is the normal direction of (001), is the direction in which the heat flux gradient is the largest. In such a hot rolling process, the gross columnar crystal can not thoroughly break due to dynamic recovery and slow re-crystallization. However, the slab columnar crystals are easy to grow in the direction of heat flux, and form gross columnar crystals having a certain orienting relation, resulting in inhomogeneous deformations in a rolling process, the center in sheet thickness is fiber texture primarily after hot rolling process, and austenite and ferrite have no phase transition in subsequent process, and will not re-crystallize in the following cold rolling and annealing process, which does not make the homogeneity of the texture eliminated, and leaving behind to the finished product, finally forming accidented corrugated defects.

The conventional methods for treating corrugated defects are mainly as follows: by utilizing electromagnetic stirring, the equiaxed crystal ratio in the slab may be improved, for example, in Japanese Patent Application Laid-open No. 49-39526; by adding the contents of carbon and manganese into steel, the phase transiting temperature in hot rolling process may be reduced, for example, in Japanese Patent Application Laid-open No. 48-49617, Chinese Patent Application CN10127519, CN1548569 and CN101139681 etc.; by utilizing low temperature pouring, the equiaxed crystal ratio in the slab may be improved, for example, in Japanese Patent Application Laid-open No. 53-14609 and No. 2-192853; by increasing furnace tap temperature of the slab, adjusting heating-up speed of the slab, controlling end-rolling temperature in a planishing process, and controlling the degree of reduction of the first and the last pass in the hot rolling process, the strip may re-crystallize sufficiently, for example, in Japanese Patent Application Laid-open No. 49-27420, No. 49-38813, No. 53-2332, No. 61-69923, Chinese Patent Application CN1548569; and by utilizing a normalized process, the strip may re-crystallize sufficiently, for example, in Japanese Patent Application Laid-open No. 61-127817, etc. In particular, CN1611616 relates to a method of manufacturing cold-rolled non-oriented electrical steel, including steps of continuously casting blanks, hot-rolling, cold rolling and then annealing thin slabs, to achieve high proportions of recrystallisation.

The above-mentioned methods may be used solely or simultaneously depending on technology, cost and the demands on the magnetism of the finished product and surface. These methods have characteristics and requirements described below, respectively.

By utilizing electromagnetic stirring, the equiaxed crystal ratio in the slab may be improved. This method utilizes electromagnetic stirring, the columnar crystals may break under electromagnetic force, and therefore, the effect thereof is the most effective. This method will remarkably reduce the columnar crystal ratio in the slab and improve the equiaxed crystal ratio in the temperature in a planishing process, and controlling the degrees of reduction of the first and the last pass in the hot rolling process, the gross columnar crystals in the slab may break, so as to prohibit the development of the gross deformation crystal grains as well as to make the strip re-crystallized sufficiently. The main disadvantage of this method is that increasing the furnace tap temperature of the slab will make the impurities such as MnS, AlN etc., solutionized intensively, thus make the magnetism of the finished strip worse. Meanwhile, in order to ensure the re-crystallization effect of the strip, the contents of impurity elements such as S, N etc., in steel are strictly demanded. Also, improving the degrees of reduction of the first and the last pass in the hot rolling process is restricted by self-capability of a rolling mill.

By utilizing the normalized process, the strip may re-crystallize sufficiently. When the single cold rolling method is utilized, the steel grade that has a high content of silicon needs to carry out the normalized process, one of the objects is to increase the re-crystallizing ratio in the hot rolling sheet, so as to avoid the generation of the corrugated defects. The main disadvantage of this method is that the manufacturing cost is very high, which is not applied in low or middle steel grade silicon steel of which the additional value is relatively low.

### Disclosure of the Invention

The object of the present invention is to provide a non-oriented electrical steel sheet without the corrugated defect and a manufacturing method thereof. The manufacture of a middle steel grade non-oriented electrical steel sheet without corrugated defect can be accomplished, which has advantages of easy operation, low cost, energy conservation and environmental protection, and excellent magnetism, by strictly controlling the cooling speed of the slab in continuous casting and pouring process, the temperature difference in the length direction of the slab in the heating furnace, and by controlling the temperature drop before planishing the slab. Meanwhile, the casting speed of the slab in continuous casting and pouring process is normal, so that the relatively high superheat of the liquid steel can be maintained, and the relatively low furnace tap temperature of the slab, and normal end-rolling temperature and coiling temperature etc., can be maintained in the hot rolling and steel reheating process, so that the strip in the hot rolling process does not need to carry out a normalized process.

In order to obtain the above-described object, the technical solution of the present invention is that
a middle steel grade non-oriented electrical steel sheet without the corrugated defect, wherein the weight percentage of the chemical composition thereof is that C is no more than 0.005%, Si is 1.2-2.2%, Mn is 0.2-0.4%, P is no more than 0.2%, S is no more than 0.005%, Al is 0.2-0.6%, N is no more than 0.005%, O is no more than 0.005%, balance Fe and inevitable impurities; where the equiaxed crystal ratio in the steel sheet is at least 43%, and where the thickness of the sheet is 2.0mm - 2.8mm.

In the sub-designs of the present invention,

C is no more than 0.005%.C is an element for strongly inhibiting the growth of crystal grains, which is easy to result in the increase of iron loss of a strip, producing the serious magnetic aging. Meanwhile, C may further widen γ phase, and increase the transition amount between α phase and γ phase when in the normalized process, so as to reduce Acl point notably, and to fine crystallizing structure. Therefore, C is necessary to be controlled to no more than 0.005%.

Si is 1.2%-2.2%. Si is an effective element for increasing the electrical resistivity of the steel. If the content of Si is lower than 1.2%, the electromagnetic performance of the steel is not good, whereas if the content of Si is higher than 2.2%, phase change will not occur in the hot rolling process, and the cold-working performance is not good.

Al is 0.2%-0.6%. Al is an effective element for increasing the electrical resistivity of the steel. If the content of Al is lower than 0.2%, the electromagnetic performance is not stable, whereas if the content of Al is higher than 0.6%, the smelting and pouring process will become difficult, thus increasing the manufacturing cost.

Mn is 0.2%-0.4%. Like the elements Si and Al, Mn may increase the electrical resistivity of the steel, as well as improve the surface state of the electrical steel, so it is necessary to add no less than 0.2% of Mn. While the content of Mn is higher than 0.4%, the smelting and pouring process will become difficult, thus increasing the manufacturing cost.

P is no more than 0.2%. Adding some phosphorus into steel can improve the workability of steel sheet, but if the content of phosphorus is more than 0.2%, it instead makes the cold rolling workability of steel plate deteriorated.

S is no more than 0.005%. If the content of S is more than 0.005%, the deposition amount of sulfide such as MnS, will increase greatly, thus strongly preventing crystal grains growing and making iron loss worse.

N is no more than 0.005%. If the content of N is more than 0.005%, the deposition amount of nitride such as AlN, will increase greatly, thus strongly preventing crystal grains growing and making iron loss worse.

O is no more than 0.005%. If the content of O is more than 0.005%, the impurity amount of oxidate such as Al₂O₃, will increase greatly, thus strongly preventing crystal grains growing and making iron loss worse.

A method for manufacturing a non-oriented electrical steel sheet without corrugated defect of the present invention comprises the following steps:
1) the weight percentage of the chemical composition of non-oriented electrical steel sheet is that C <0.005%, Si is 1.2-2.2%, Mn is 0.2-0.4%, P <0.2%, S <0.005%, Al is 0.2-0.6%, N <0.005%, O <0.005%, balance Fe and inevitable impurities, in accordance with the above chemical composition, a slab is obtained by hot metal preprocessing, smelting with converter, RH refining, and continuous casting and pouring, where the casting speed is between 0.95m/min and 1.07m/min; wherein a secondary cooling in amount is controlled, the water flowrate of cooling water is controlled to 100-190 l/min, the average superheat of liquid steel in the continuous casting process is controlled to 10-45°C;
2) the slab is heated and hot rolled;
   the furnace tap temperature of the slab is 1050-1150°C, the temperature difference between the random two points in the length direction when the slab is heated, is lower than 25°C, the hot rolling process includes a rough rolling process and a planishing process, the entry temperature in the planishing process is no lower than 970°C; the residence time of the slab in the after-firing zone is no less than 45mins; wherein the rolling sheet is rolled to a thickness of 2.0mm - 2.8mm; wherein the end rolling temperature is controlled to about 850°C, and the coiling temperature is controlled to between 563°C and about 600°C;
3) the finished non-oriented electrical steel sheet is obtained by acid pickling, cold rolling, annealing and coating.

The middle steel grade non-oriented electrical steel sheet without corrugated defect of the present invention and the manufacturing method thereof comprise the following steps:
The average superheat of liquid steel in the pouring process is controlled to 10-45°C. In the continuous casting and pouring process, the water flowrate of cooling water is adjusted to 100-190 l/min, so as to improve the equiaxed crystal ratio in the slab, avoiding columnar crystals in the slab gross and growing.

Relatively low temperature, which affects the surface temperature of the slab so as to make the strip re-crystallized insufficiently, should be avoided. Therefore, the temperature difference between the random two points in the length direction when the slab is heated, is controlled to be lower than 25°C; the temperature difference between the watermark points of the slab is limited within 25°C, meanwhile the residence time of the slab in after-firing zone should be no less than 45 min, so as to ensure uniform heating, making the temperatures of both surfaces of the slab close.

The furnace tap temperature of the slab can be reduced to no higher than 1150°C, avoiding the impurities such as MnS, AlN etc., solutionized intensively, which thus making the magnetism of the finished strip worse. Hot rolling sheet is rolled to have a thickness of 2.0mm-2.8mm. Before the rough rolling process and the planishing process, hot tops are respectively utilized to thermal insulate the slab and the intermediate billet, the entry temperature in the planishing process is controlled to no lower than 970°C so as to facilitate sufficient re-crystallization, and the end-rolling temperature is controlled to about 850 °C, the coiling temperature is controlled to about 600 °C.

The hot rolling is rolled to thick strip that has a thickness of 0.5mm, and then is annealed continuously in a dry atmosphere. In the continuous annealing process, the electromagnetic performance of the steel is further improved by warming up the finished strip quickly in a preheating zone, in which the heat-up speed is no less than 1000°C/min, and by controlling the atmosphere mode in furnace.

Basing on the controlling demand on the composition of the present invention, after the extent of silicon in the steel exceeds 2.2%, when an electromagnetic stirring is not utilized or a slightly electromagnetic stirring is utilized, since the content of silicon is relatively high, the columnar crystal in the slab is growing and gross, and the electromagnetic stirring force is not enough to break the columnar crystals, and a part of the broken columnar crystals will still polymerize and grow once again, so that making the ratio of fine equiaxed crystals in the slab is relatively low while the ratio of gross and growing columnar crystals is relatively high. Therefore, it is necessary to improve electromagnetic stirring intensity so as to control the corrugated defects in the surface of the finished strip.

In the present invention, when the content of silicon is less than 2.2%, the content of silicon does not affect the growth of the columnar crystal as greatly as the cooling speed of the slab, therefore, the water flowrate of cooling water in the continuous casting process can be adjusted to reduce the heat flux gradient of the slab in the growing direction of the columnar crystal, so that the ratio of gross and growing columnar crystals can be reduced effectively. Further, considering the temperature of the slab at the location where the slab contacts the roller table is relatively low in the slab heating process, which affects the re-crystallization of the fiber texture in the interior of the slab, not making the homogeneity of the texture eliminated and leaving behind to the finished product, therefore, it is necessary to strictly control the temperature of the watermark point of the slab. The main reason on improving the entry temperature in the planishing process is to facilitate the break and elimination of the columnar crystals in the rolling process and improve the re-crystallization ratio of the fiber texture in the hot rolling strip.

Also, since the content of silicon is no more than 1.2%, the phase change from γ phase to α phase in the hot rolling process is sufficient, the corrugated defects will not occur in the surface of the subsequent finished product.

Also, if two or three pairs of electromagnetic stirring rolls are utilized, the columnar crystals in the slab may be broken due to highly electromagnetic stirring force, as possible as to transit to fine equiaxed crystals, so as to improve the equiaxed crystal ratio in the slab greatly; or the phase change from γ phase to α phase happens in the interior of the slab by increasing the furnace tap temperature of the slab in the heat process greatly, meanwhile the re-crystallization of the slab is improved by utilizing high temperature status to enlarge the re-crystallizing structure in the interior of the slab. Except for the great increasement in the aspect of equipment investment and energy consumption, it is more important that the electromagnetic stirring technology is hard to match the superheat of the liquid steel precisely, if the superheat of the liquid steel is controlled improperly, the controlling effect of the electromagnetic stirring is not stable, which is hard to obtain the expecting effect; and by increasing the furnace tap temperature of the slab, the heating load distribution in the heating furnace will forward, making high temperature time zone relatively long, which affects the magnetism of the finished strip. This method is easy to result in mass defect at the edge of the strip with respect to high-silicon steel grade.

Under the condition of the special chemical composition of the present invention, the water flowrate of cooling water in the continuous casting process can be adjusted to reduce the heat flux gradient of the slab in the growing direction of the columnar crystal, so that the ratio of gross and growing columnar crystals can be reduced effectively. It is more important that this method is substantially affected by the change in the superheat of the liquid steel, so the range of application is relatively wide. Meanwhile, the adjustment on the water flowrate of cooling water is very simple and controllable, so the difficulty in implementation is low, the stability is good. Further, the equipment load may be reduced by utilizing lower furnace tap temperature of the slab, avoiding the deposition of fine impurities in the steel and affecting the magnetism of final product. If the lower temperature is used to heat the slab, the temperature at the watermark points in the slab may be adjusted to increase re-crystallizing ratio of the fiber texture of the slab in the hot rolling process, and to improve the homogeneity of the texture of the slab in the hot rolling strip, which facilitates to the corrugated defects in the surface of the finished strip.

### Brief Description of Drawings

Fig. 1 is a schematic view of the relation between the water flowrate of the cooling water and the equiaxed crystal ratio in the slab.
Fig. 2 is a schematic view of the relation between the entry temperature in the hot rolling and planishing process and the incidence of the corrugated defects in a finished product.
Fig. 3 is a schematic view of the relation between the furnace tap temperature of the slab and the magnetism of the finished product.
Fig. 4 is a picture of a metallographic structure of a strip in hot rolling process corresponding to a watermark point temperature of 20°C.
Fig. 5 is a picture of a metallographic structure of a strip in hot rolling process corresponding to a watermark point temperature of 35°C.

### Detailed Description of the Invention

Hereinafter, the present invention will be described in connection with the embodiments and drawings.

### First Embodiment

The chemical composition of the tundish liquid steel in the continuous casting process is controlled as follows: C is 0.001%, Si is 1.22%, Mn is 0.25%, P is 0.02%, S is 0.003%, Al is 0.33%, N is 0.001%, O is 0.004%, balance Fe and inevitable impurities. The average superheat of the liquid steel is 34.6°C, the casting speed is 1.07m/min, the water flowrate of the cooling water is 185 l/min, the temperature drop speed of the slab is 11.6min/°C, the surface temperature of the slab at the outlet of a caster is 710 °C and the equiaxed crystal ratio is 43%.In the heating furnace, the temperature difference between the watermark points is 22°C, the residence time in after-firing zone of the slab is 46 minutes. The rolling process will be carried out after heating for 3h at 1125°C, the temperature at the inlet in planishing process is 978°C, the end-rolling temperature is 856°C and the coiling temperature is 567°C. The hot rolling sheet is rolled to 0.5mm thickness of strip with the single cold rolling method, and then is annealed continuously in a dry atmosphere. Corrugated defects are not generated in the surface of the finished strip, the iron loss is 4.743 W/kg, and the magnetic induction is 1.727T.

### Second Embodiment

The chemical composition of the tundish liquid steel in the continuous casting process is controlled as follows: C is 0.002%, Si is 1.42%, Mn is 0.30%, P is 0.06%, S is 0.002%, Al is 0.25%, N is 0.002%, O is 0.002%, balance Fe and inevitable impurities. The average superheat of the liquid steel is 31.4°C, the casting speed is 1.04m/min, the water flowrate of the cooling water is 175 l/min, the temperature drop speed of the slab is 9.6 min/°C, the surface temperature of the slab at the outlet of a caster is 680°C and the equiaxed crystal ratio is 57%.In the heating furnace, the temperature difference between the watermark points is 22°C, the residence time in after-firing zone of the slab is 48 minutes. The rolling process will be carried out after heating for 3h at 1135°C, the temperature at the inlet in planishing process is 973°C, the end-rolling temperature is 853°C and the coiling temperature is 563 °C .The hot rolling sheet is rolled to 0.5mm thickness of strip with the single cold rolling method, and then is annealed continuously in a dry atmosphere. Corrugated defects are not generated in the surface of the finished strip, the iron loss is 3.130 W/kg, and the magnetic induction is 1.741T.

### Third Embodiment

The chemical composition of the tundish liquid steel in the continuous casting process is controlled as follows: C is 0.002%, Si is 1.49%, Mn is 0.49%, P is 0.02%, S is 0.003%, Al is 0.59%, N is 0.001%, O is 0.002%, balance Fe and inevitable impurities. The average superheat of the liquid steel is 28.7°C, the casting speed is 0.99m/min, the water flowrate of the cooling water is 189 l/min, the temperature drop speed of the slab is 8.7 min/°C, the surface temperature of the slab at the outlet of a caster is 660°C and the equiaxed crystal ratio is 63%.In the heating furnace, the temperature difference between the watermark points is 24°C, the residence time in after-firing zone of the slab is 53 minutes. The rolling process will be carried out after heating for 3h at 1102°C, the temperature at the inlet in planishing process is 983°C, the end-rolling temperature is 854°C and the coiling temperature is 575°C .The hot rolling sheet is rolled to 0.5mm thickness of strip with the single cold rolling method, and then is annealed continuously in a dry atmosphere. Corrugated defects are not generated in the surface of the finished strip, the iron loss is 3.559 W/kg, and the magnetic induction is 1.737T.

### Fourth Embodiment

The chemical composition of the tundish liquid steel in the continuous casting process is controlled as follows: C is 0.001%, Si is 2.12%, Mn is 0.25%, P is 0.01%, S is 0.002%, Al is 0.36%, N is 0.001%, O is 0.004%, balance Fe and inevitable impurities. The average superheat of the liquid steel is 31.2°C, the casting speed is 0.95m/min, the water flowrate of the cooling water is 173 l/min, the temperature drop speed of the slab is 13.2 min/°C, the surface temperature of the slab at the outlet of a caster is 680°C and the equiaxed crystal ratio is 59%. In the heating furnace, the temperature difference between the watermark points is 20°C, the residence time in after-firing zone of the slab is 48 minutes. The rolling process will be carried out after heating for 3h at 1097°C, the temperature at the inlet in planishing process is 972°C, the end-rolling temperature is 844°C and the coiling temperature is 583°C. The hot rolling sheet is rolled to 0.5mm thickness of strip with the single cold rolling method, and then is annealed continuously in a dry atmosphere. Corrugated defects are not generated in the surface of the finished strip, the iron loss is 2.833 W/kg, and the magnetic induction is 1.726T.

### Comparative Example

The chemical composition of the tundish liquid steel in the continuous casting process is controlled as follows: C is 0.001%, Si is 1.47%, Mn is 0.32%, P is 0.02%, S is 0.003%, Al is 0.25%, N is 0.002%, O is 0.002%, balance Fe and inevitable impurities. The average superheat of the liquid steel is 28.9°C, the casting speed is 1.03m/min, the water flowrate of the cooling water is 257 l/min, the temperature drop speed of the slab is 17.4 min/°C, the surface temperature of the slab at the outlet of a caster is 580°C and the equiaxed crystal ratio is 28%. In the heating furnace, the temperature difference between the watermark points is 37°C, the residence time in after-firing zone of the slab is 41 minutes. The rolling process will be carried out after heating for 3h at 1153°C, the temperature at the inlet in planishing process is 947°C, the end-rolling temperature is 847°C and the coiling temperature is 567°C. The hot rolling sheet is rolled to 0.5mm thickness of strip with the single cold rolling method, and then is annealed continuously in a dry atmosphere. The percentage of the generation of corrugated defects in the surface of the finished strip is as high as no less than 90%, the iron loss is 3.273 W/kg, and the magnetic induction is 1.736T.

Fig. 1 shows the relation between the water flowrate of the cooling water and the equiaxed crystal ratio in the slab. As seen in Fig.l, on the premise of not utilizing an electromagnetic stirring, by decreasing the water flowrate of the cooling water and strictly controlling it to no more than 190 l/min, the equiaxed crystal ratio in the slab is improved remarkably. In the embodiments, the equiaxed crystal ratio in the slab may be controlled when the superheat of the liquid steel is relatively high. In the fourth embodiment of these embodiments, when the water flowrate of the cooling water is 173 l/m, the equiaxed crystal ratio in the slab is up to 59%, in the comparative example, when the water flowrate of the cooling water is 257 l/min, the equiaxed crystal ratio in the slab is only 28%. Also, in the third embodiment, the control of the equiaxed crystal ratio in the slab is better, up to 63%.

Fig. 2 shows the relation between the entry temperature in the hot rolling and planishing process and the incidence of the corrugated defects in a finished product. It is indicated in accordance with the statistical results that by increasing the entry temperature in the hot rolling and planishing process and up to more than 970°C, because the re-crystallizing ratio of the fiber texture of the slab in the hot rolling process is increased remarkably, the incidence of the corrugated defects in the finished strip may be reduced greatly. In the comparative example, the entry temperatures in the hot rolling and planishing process of most of strips are less than 970°C, the percentage of the generation of corrugated defects in the surface of the finished strip is as high as no less than 90%. In several embodiments, most of the entry temperatures in the hot rolling and planishing process of strips are more than 970°C, corrugated defects are not generated in the surface of the finished strip, respectively.

Fig. 3 shows the relation between the furnace tap temperature of the slab and the magnetism of the finished product. The higher the furnace tap temperature of the slab is, the worse the magnetism of the finished product is.

Figs. 4 and 5 are metallographic structures of strips in hot rolling process corresponding to different watermark point temperatures. The watermark point temperatures are all less than 25°C in the first to fourth embodiments, so re-crystallizing structures of the strips in the hot rolling process are very homogeneous, the fiber textures disappear completely, whereas in the comparative example, the temperature at the watermark point is as high as 37 °C, the fiber texture of the strip in the hot rolling process is clear, which is hard to re-crystallized in the period of the subsequent cold rolling and annealing process, not being able to destroy the homogeneity of the structures and leaving behind to the finished product, finally forming accidented corrugated defects.

## Claims

1. A non-oriented electrical steel sheet without corrugated defect, wherein the weight percentage of the chemical composition thereof is that C <0.005%, Si is 1.2-2.2%, Mn is 0.2-0.4%, P <0.2%, S <0.005%, Al is 0.2-0.6%, N <0.005%, O <0.005%,balance Fe and inevitable impurities; where the equiaxed crystal ratio in the steel sheet is at least 43%, and where the thickness of the sheet is 2.0mm-2.8mm.

2. A method for manufacturing a non-oriented electrical steel sheet without corrugated defect of Claim 1, comprising the following steps:
1) the weight percentage of the chemical composition of non-oriented electrical steel sheet is that C <0.005%, Si is 1.2-2.2%, Mn is 0.2-0.4%, P <0.2%, S <0.005%, Al is 0.2-0.6%, N <0.005%, O <0.005%, balance Fe and inevitable impurities, in accordance with the above chemical composition, a slab is obtained by hot metal preprocessing, smelting with converter, RH refining, and continuous casting and pouring, where the casting speed is between 0.95m/min and 1.07m/min;
wherein a secondary cooling water amount is controlled, the water flowrate of cooling water is controlled to 100-190 l/min, the average superheat of liquid steel in the continuous casting process is controlled to 10-45°C;
2) the slab is heated and hot rolled;
wherein the furnace tap temperature of the slab is 1050-1150°C, the temperature difference between the random two points in the length direction when the slab is heated, is lower than 25°C, the hot rolling process includes a rough rolling process and a planishing process, the entry temperature in the planishing process is no lower than 970°C; the residence time of the slab in the after-firing zone is no less than 45mins; wherein the rolling sheet is rolled to a thickness of 2.0mm - 2.8mm; wherein the end-rolling temperature is controlled to about 850°C, and the coiling temperature is controlled to being less than 600°C;
3) the finished non-oriented electrical steel sheet is obtained by acid pickling, cold rolling, annealing and coating.

## Patentansprüche

1. Nichtorientierte elektrische Stahlplatte ohne Wellungsdefekt, wobei die Gewichtsprozente der chemischen Zusammensetzung davon C < 0,005%, Si 1,2 - 2,2%, Mn 0,2 - 0,4%, P < 0,2%, S < 0,005%, Al 0,2 - 0,6%, N < 0,005%, O < 0,005%, Rest Fe und unvermeidbare Verunreinigungen sind; wobei das gleichachsige Kristallverhältnis in der Stahlplatte mindestens 43% beträgt und wobei die Dicke der Platte 2,0 mm - 2,8 mm beträgt.

2. Verfahren zur Herstellung einer nichtorientierten elektrischen Stahlplatte ohne Wellungsdefekt nach Anspruch 1, umfassend die folgenden Schritte, wobei:
1) der Gewichtsprozentsatz der chemischen Zusammensetzung der nichtorientiertem elektrischen Stahlplatte C < 0,005%, Si 1,2 - 2,2%, Mn 0,2 - 0,4%, P < 0,2%, S < 0,005%, Al 0,2 - 0,6%, N < 0,005%, O < 0,005%, Rest Fe und unvermeidliche Verunreinigungen beträgt, gemäß der obigen chemischen Zusammensetzung, eine Bramme durch Vorverarbeitung von heißem Metall, Schmelzen mit Wandler, RH-Raffinieren und durch kontinuierliches Gießen und Eingießen erhalten wird, wobei die Gießgeschwindigkeit zwischen 0,95 m/min und 1,07 m/min beträgt;
wobei eine sekundäre Kühlwassermenge gesteuert wird, die Wasserdurchflussrate des Kühlwassers auf 100-190 l/min gesteuert wird, die durchschnittliche Überhitzung des flüssigen Stahls im kontinuierlichen Gießverfahren auf 10-45 °C gesteuert wird;
2) die Bramme erwärmt und warmgewalzt wird;
wobei die Ofenabstichtemperatur der Bramme 1050 - 1150 °C beträgt, die Temperaturdifferenz zwischen den zufälligen zwei Punkten in Längenrichtung, wenn die Bramme erwärmt wird, kleiner als 25 °C ist, der Warmwalzprozess einen Grobwalzprozess und einen Planierprozess aufweist, die Eintrittstemperatur in den Planierprozess nicht kleiner als 970 °C ist;
die Verweilzeit der Bramme in der Nachbrennzone mindestens 45 Minuten beträgt;
wobei die Walzplatte auf eine Dicke von 2,0 mm-2,8 mm gewalzt wird;
wobei die Endwalztemperatur auf etwa 850 °C gesteuert wird und die Haspeltemperatur auf kleiner als 600 °C gesteuert wird;
3) die fertige nichtorientierte elektrische Stahlplatte durch Säurebeizen, Kaltwalzen, Glühen und Beschichten erhalten wird.

## Revendications

1. Feuille d'acier électrique non orientée sans défaut ondulé, les pourcentages en poids de la composition chimique de celle-ci étant que C < 0,005 %, Si est de 1,2 à 2,2 %, Mn est de 0,2 à 0,4 %, P < 0,2 %, S < 0,005 %, Al est de 0,2 à 0,6 %, N < 0,005 %, O < 0,005 %, le reste étant Fe et des impuretés inévitables ; le rapport des cristaux équiaxes dans la feuille d'acier étant d'au moins 43 %, et l'épaisseur de la feuille étant de 2,0 mm à 2,8 mm.

2. Procédé pour la fabrication d'une feuille d'acier électrique non orientée sans défaut ondulé selon la revendication 1, comprenant les étapes suivantes :
1) les pourcentages en poids de la composition chimique de la feuille d'acier électrique non orientée étant que C < 0,005 %, Si est de 1,2 à 2,2 %, Mn est de 0,2 à 0,4 %, P < 0,2 %, S < 0,005 %, Al est de 0,2 à 0,6 %, N < 0,005 %, O < 0,005 %, le reste étant Fe et des impuretés inévitables, conformément à la composition chimique ci-dessus, une plaque est obtenue par prétraitement de métal à chaud, fusion avec un convertisseur, affinage RH (Ruhrstahl Heraeus), et coulée et versement en continu, la vitesse de coulée étant comprise entre 0,95 m/min et 1,07 m/min ;
une quantité d'eau de refroidissement secondaire étant réglée, le débit d'eau de refroidissement étant réglé de 100 à 190 l/min, la surchauffe moyenne d'acier liquide dans le procédé de coulée continue étant réglée de 10 à 45 °C ;
2) la plaque est chauffée et laminée à chaud ;
la température de percée de four de la plaque étant de 1050 à 1150 °C, la différence de température entre deux points aléatoires dans la direction longitudinale lorsque la plaque est chauffée, étant inférieure à 25 °C, le procédé de laminage à chaud comportant un procédé de laminage grossier et un procédé d'aplanissement, la température d'entrée dans le procédé d'aplanissement étant supérieure ou égale à 970 °C ; le temps de séjour de la plaque dans la zone d'après-cuisson étant supérieur ou égal à 45 min ;
la feuille laminée étant laminée jusqu'à une épaisseur de 2,0 mm à 2,8 mm ;
la température de fin de laminage étant réglée à environ 850 °C, et la température d'enroulement étant réglée de sorte à être inférieure à 600 °C ;
3) la feuille d'acier électrique non orientée finie est obtenue par décapage acide, laminage à froid, recuisson et revêtement.
